

1

3,672,940

**PROCESS FOR CHEMICALLY DEPOSITING NICKEL  
ON A SYNTHETIC RESIN BASE MATERIAL**

Kiyotaka Funada, Chigasaki, Takashi Shinohara, Yokohama, and Hiroko Imai, Tokyo, Japan, assignors to Nihon Kagaku Kizai Kabushiki Kaisha, Tokyo, Japan No Drawing. Filed Aug. 3, 1970, Ser. No. 60,628

Claims priority, application Japan, Aug. 8, 1969,

44/62,687

Int. Cl. B44d 1/092; C23c 3/02

U.S. Cl. 117—47 A

7 Claims

**ABSTRACT OF THE DISCLOSURE**

A process for the chemical deposition of nickel on a synthetic resin base material, characterized by etching the resin base material in a new etching solution containing a palladium compound as the additive thereby eliminating the conventional sensitizing and activating treatments, and chemically depositing nickel on the etched resin base material from a new chemical nickel plating bath containing as the additives a water-soluble lead compound and a second reducing compound such as ascorbic acid, thereby obtaining the new plating bath having a better plating capability and longer lifetime.

This invention relates to a process for forming a nickel coating on a synthetic resin base material.

A process for coating a synthetic resin base material with nickel has greatly been improved and consequently the adhesion of a nickel coating to a resinous material has been improved. Thus, such nickel coated synthetic resin articles have been in great demand instead of die-cast zinc and aluminum articles for the same use in many industrial fields.

However, since the electroplating of a synthetic resin article according to such a conventional process requires not a few preliminary steps of rendering the resinous article electrically conductive, it will cost a lot of money for industrial equipments if industrialized and will need operators of long-period experience to be carried out satisfactorily. Thus there is a tendency that even operators skilled in the art produce coated articles where the coating is not securely attached to the base article and is not uniformly formed thereon. In addition to these disadvantages, the conventional process will produce nickel coatings which have clouding with non-uniform thickness.

A conventional process for forming chemical copper or nickel coatings, which is now prevalently in use usually as the preliminary one for the subsequent electroplating, typically comprises as many as 16 steps shown hereunder:



2

The chemical coating thus washed with water is usually followed by electroplating to increase the coating in thickness.

In the practice of said conventional, chemical coating, a synthetic resin base material is first degreased with a weakly alkaline solution, washed with water and immersed in an etching solution consisting of chromic acid and sulfuric acid to provide the base material with receptivity for a metal coating to be formed thereon. In this treatment the composition and temperature of the etching bath as well as the time of immersion therein should properly be controlled to obtain a satisfactory etching. If the etched base material is immersed in the subsequent sensitizing bath containing stannous ion without thoroughly removing the chromium ion adsorbed on the surface thereof during the etching treatment, the still remaining chromium ion will hinder the stannous ion from being adsorbed on the base material from the sensitizing bath and will oxidize the stannous ion present in the sensitizing bath thereby accelerating the using up of this bath. Thus, the etched base material should be washed with water usually three times to remove the chromium ion therefrom before immersed in the subsequent sensitizing bath.

The sensitizing bath usually consists of a dilute solution of stannous chloride in hydrochloric acid and should be such that the stannous ion therefrom is allowed to be adsorbed on the sensitized base material in an amount necessary and sufficient to reduce palladium ion to be attached to the base material in the following activating step. An insufficient amount of the stannous ion adsorbed will be a cause for forming a skip plating, and the introduction of excessive stannous ion into the activating bath will reduce unnecessarily too much of the palladium ion present therein thereby promoting the degradation of this bath. And further, if the activated base material is carried into a chemical plating bath together with the unnecessarily reduced, minutely particulate metallic palladium attached thereto, a nickel coating with a rough surface will be formed on the base material.

As the activating bath, a bath consisting of a dilute solution of palladium chloride in hydrochloric acid will commonly be used when a chemical nickel coating is to be obtained. The stannous ion adsorbed on the base material from the sensitizing bath, when the base material is immersed in the activating bath containing palladium ion, will reduce the palladium ion to metallic palladium in fine particulate form which is then securely adsorbed on the base material. A chemical nickel skip plating will be formed if the amount of metallic palladium adsorbed is insufficient, while undesirable palladium ion, if carried into a chemical nickel plating bath with the base material, will function as catalytic nuclei thereby depositing and suspending nickel in the bath or, in some cases, decomposing the bath with the result that it cannot be used any further.

There have hitherto been proposed various processes for the formation of a chemical nickel coating, in which processes some of the above-mentioned conventional troublesome steps are eliminated. However, many of these processes have their own disadvantages and they are therefore not considered to be practicable.

This invention relates to a process for forming a chemical nickel coating on a synthetic resin base material, characterized in that it uses both a new etching bath prepared by adding a very small amount of palladium ion to a conventional etching bath containing a mixed solution of sulfuric and chromic acids and a new plating bath prepared by adding a second reducing agent and an anti-decomposition agent for the plating bath to a conventional chemical nickel plating bath containing nickel and hypophosphite ions, whereby the etching and activating treat-

ments can be carried out at a time by use of the new etching bath and the sensitizing treatment can be dispensed with. Thus the process of this invention may comprise much fewer steps than the conventional ones and it usually comprises only 9 steps as shown below:



The synthetic resin base material treated by the process of this invention is then subjected to electroplating.

Chemical nickel plating baths which may be used in the practice of this invention, are prepared by adding ascorbic acid or a salt thereof as a second reducing agent and a water-soluble lead compound as an anti-decomposition agent for the bath to a conventional acidic or alkaline bath containing nickel and hypophosphite ions together with an organic acid, boron compound and other suitable compounds as a complexing and/or buffer agent.

When palladium ion is introduced in such a chemical plating bath containing nickel and hypophosphite ions, the hypophosphite ion will, with aid of the catalytic action of metallic palladium, cause the following reaction:



The hydrogen atoms thus produced are adsorbed on the surface of the catalytic metal to activate the surface thereby reducing the nickel ion and depositing metallic nickel as indicated below:



The metallic nickel thus deposited then functions as a catalyst in the reaction (1) thereby allowing the reaction to proceed while forming a nickel coating. Thus, in order to plate with nickel a metal which is catalytically inactive in the reaction (1), the nickel is necessary to deposit on the inactive metal by means of substitution reaction or galvanization.

Such galvanization is not applicable to a synthetic resin material which is a poor electric conductor. Thus it is necessary to subject the resin material to the activating treatment in order to adsorb a catalytic material, such as metallic palladium, thereon for the subsequent deposition of nickel with aid of the catalyst as crystallizing nuclei. If the metallic palladium adsorbed on the resin material in the activating treatment is peeled off the resin material when immersed in the plating bath or if the resin material is immersed in the plating bath together with some of the activating solution of palladium still remaining on the resin material because of insufficient washing thereof with water and the solution is dispersed throughout the plating bath, the palladium thus introduced will form catalytic nuclei thereby causing such reactions as above and depositing nickel as a precipitate in the plating bath. If such nickel deposited is attached to the resin material, it will form a spotted nickel coating thereon. In addition, if the plating bath is incorporated with too much of the palladium, it will continue to deposit nickel until depletion of the nickel ion therein and it may entirely decompose. If, for too much fear of this, the resin material from the activating bath is too much repeatedly washed with water, some portions of the surface thereof will not be covered with nickel when immersed in the nickel plating

bath because the palladium once adsorbed on said portions may have been washed away by said too much washing. The foregoing is the reason why even workmen very skilled in the art cannot necessarily produce satisfactorily nickel-coated articles only.

It is considered that, in the chemical nickel plating bath according to this invention, the ascorbic acid selectively reduces the palladium ion adsorbed on the resinous base material from the etching and activating bath prior to the start of reduction of the nickel ion by the hypophosphite ion thereby preventing the palladium ion from diffusing throughout the plating bath, while the palladium ion dragged into the plating bath together with the resinous base material is occluded or caught in the lead ion, which is a negative catalyst for the reducing action of the hypophosphite ion, thereby losing its catalytic capability. The ascorbic acid may be substituted by its salt and may be used in any desired amounts.

In the plating bath according to this invention, the lead ion should preferably be contained in amounts of not more than 10 p.p.m. since the hypophosphite ion will decrease in reducing power or reducibility if too much of lead ion is present. The plating bath may be acidic or alkaline. It should preferably be at a pH value of 3 to 10 and it will decrease the rate at which nickel is deposited therefrom, when kept at a pH value of not more than 3. The optimum temperature of the plating bath when in use does not have to be changed due to the presence of ascorbic acid in the bath. The bath may thus be kept at the same suitable temperature as the conventionally used baths, when in use.

Typical etching solutions which may be used in the practice of this invention, comprise 100-900 cc./l. of conc.  $\text{H}_2\text{SO}_4$ , 0-200 cc./l. of phosphoric acid, 900-100 cc./l. of water, 5-300 g./l. (calculated as  $\text{CrO}_3$ ) of chromic acid anhydride and 0.05-5 g./l. (calculated as Pd) of a palladium salt and, preferably, 400-900 cc./l. of conc.  $\text{H}_2\text{SO}_4$ , 0-100 cc./l. of phosphoric acid, 600-100 cc./l. of water, 5-30 g./l. (calculated as  $\text{CrO}_3$ ) of chromic acid anhydride and 0.2-5 g./l. (calculated as Pd) of a palladium salt. The chromic acid anhydride may be substituted by potassium dichromate, and the palladium salt is selected from palladium chloride, palladium sulphate and sodium palladium chloride.

Typical nickel plating baths which may be used, comprise 1-18 g./l. (calculated as Ni ion) of a nickel salt, 3-40 g./l. (calculated as hypophosphite ion) of a hypophosphite, 5-100 g./l. of an organic acid, 1-50 g./l. (calculated as ascorbic acid) of an ascorbic acid type compound and 1-10 mg./l. (calculated as lead ion) of a lead salt and, preferably, 2-8 g./l. (calculated as Ni ion) of a nickel salt, 5-18 g./l. (calculated as hypophosphite ion) of a hypophosphite, 10-30 g./l. of an organic acid, 10-30 g./l. (calculated as ascorbic acid) of an ascorbic acid type compound and 2-7 mg./l. of a lead salt. The baths should be at a pH value of 3-10, preferably, 4-9. The nickel salt may be nickel sulphate, nickel chloride or the like; the hypophosphite is typically sodium hypophosphite; the ascorbic acid type compound may be ascorbic acid, sodium ascorbate or the like; and the organic acid is selected from short chain monocarboxylic acids such as acetic, propionic and butyric acids, and the salts thereof; dicarboxylic acids such as malonic, succinic and adipic acids, and the salts thereof; tricarboxylic acids such as citric acid, and the salts thereof; hydroxycarboxylic acids such as glycolic, lactic, malic and tartaric acids, and the salts thereof; and aminocarboxylic acids such as aminoacetic and aminopropionic acids, and the salts thereof. The salts of these various acids are typically the sodium, potassium, ammonium and other like salts. The lead salt is selected from lead nitrate and acetate. Together with the above-mentioned organic acids, there may be used ammonium chloride, borax and the like.

This invention will be better understood by the following examples.

## 5

## EXAMPLE 1

Test pieces (65 mm. x 40 mm. x 3 mm.) of acrylonitrile-butadiene-styrol (ABS) resin (Plating Grade, this resin being the one made by Ube Cycon Co., Ltd., Japan) were degreased with an alkali, washed with water and immersed in an etching solution at 60° C. for 15 minutes to etch them, the etching solution having the following composition:

|                                             |        |     |    |
|---------------------------------------------|--------|-----|----|
| Concentrated H <sub>2</sub> SO <sub>4</sub> | cc./l. | 500 | 10 |
| Water                                       | cc./l. | 500 |    |
| Chromic acid anhydride                      | g./l.  | 15  |    |
| Palladium chloride                          | g./l.  | 0.5 |    |

Some of the thus-etched test pieces, after washed with water, were then immersed in 200 cc. of a novel chemical plating bath at 40° C. for 5 minutes in an attempt to form a nickel coating thereon, the novel plating bath having the following composition:

|                         |        |     |    |
|-------------------------|--------|-----|----|
| Nickel sulphate         | g./l.  | 20  | 20 |
| Sodium hypophosphite    | g./l.  | 15  |    |
| Adipic acid             | g./l.  | 10  |    |
| L-ascorbic acid         | g./l.  | 10  |    |
| Lead nitrate            | mg./l. | 5.5 |    |
| pH (adjusted with NaOH) |        | 6.0 | 25 |

For comparison, the rest of the etched test pieces, after washed with water, were then immersed in 200 cc. of a conventional chemical plating bath at the same temperature for the same time as above in an attempt to form a nickel coating thereon, the conventional bath having the following composition:

|                         |        |     |
|-------------------------|--------|-----|
| Nickel sulphate         | g./l.  | 20  |
| Sodium hypophosphite    | g./l.  | 15  |
| Adipic acid             | g./l.  | 10  |
| L-ascorbic acid         | g./l.  | —   |
| Lead nitrate            | mg./l. | —   |
| pH (adjusted with NaOH) |        | 6.0 |

As seen from the above, the conventional bath had the same composition as the novel one except that the former did not contain L-ascorbic acid and lead nitrate.

The results obtained were as follows:

The etched test pieces immersed in the novel bath were uniformly coated with nickel on the entire surface, during which the bath was kept transparent. On the other hand, those immersed in the conventional bath were dotted with nickel on the surface while this bath produced dark-colored precipitates.

## EXAMPLE 2

The procedure of Example 1 was repeated, but using the following etching solution and conventional and novel baths under the following operational conditions:

|                                             |        |     |    |
|---------------------------------------------|--------|-----|----|
| Etching solution:                           |        |     |    |
| Concentrated H <sub>2</sub> SO <sub>4</sub> | cc./l. | 800 |    |
| Water                                       | cc./l. | 200 | 55 |
| Chromic acid anhydride                      | g./l.  | 10  |    |
| Palladium sulphate                          | g./l.  | 0.5 |    |
| Temp. of the solution                       | °C.    | 40  |    |
| Time of immersion                           | min.   | 5   | 60 |

## CHEMICAL NICKEL PLATING BATHS

|                                     | Conventional bath | Novel bath |    |
|-------------------------------------|-------------------|------------|----|
| Nickel sulphate, g./l.              | 16                | 16         |    |
| Sodium hypophosphite, g./l.         | 11                | 11         | 65 |
| Citric acid, g./l.                  | 6                 | 6          |    |
| Borax, g./l.                        | 2.5               | 2.5        |    |
| L-ascorbic acid, g./l.              | None              | 3          |    |
| Lead acetate, mg./l.                | None              | 7          |    |
| pH of the bath (adjusted with NaOH) | 8.0               | 8.0        |    |
| Temp. of the bath, °C.              | 30                | 30         |    |
| Time of immersion, min.             | 3                 | 3          | 70 |

The test pieces from the novel bath had a uniform nickel coating formed all over the initial etched surface thereof while the bath was kept transparent during the time of immersion of the test pieces therein; and, on the

other hand, the test pieces from the conventional bath had a surface which was dotted with nickel from the bath while the bath remained limpid during the time of immersion of the test pieces.

5

## 6

The procedure of Example 1 was followed, but using the following etching solution and novel and conventional baths under the following operational conditions:

Etching solution:

|                                             |        |     |
|---------------------------------------------|--------|-----|
| Concentrated H <sub>2</sub> SO <sub>4</sub> | cc./l. | 500 |
| Water                                       | cc./l. | 500 |
| Potassium dichromate                        | g./l.  | 10  |
| Sodium palladium chloride                   | g./l.  | 1   |
| Temp. of the solution                       | °C.    | 60  |
| Time of immersion                           | min.   | 10  |

## CHEMICAL NICKEL PLATING BATHS

|                                     | Conventional | Novel |
|-------------------------------------|--------------|-------|
| Nickel sulfate, g./l.               | 20           | 20    |
| Sodium hypophosphite, g./l.         | 15           | 15    |
| Sodium, succinate g./l.             | 15           | 15    |
| L-ascorbic acid, g./l.              | None         | 30    |
| Lead acetate, mg./l.                | None         | 10    |
| pH of the bath (adjusted with NaOH) | 4.0          | 4.0   |
| Temp. of the bath, °C.              | 60           | 60    |
| Time of immersion, min.             | 3            | 3     |

The test pieces immersed in the novel bath were uniformly coated with nickel on the entire surface while the bath was kept transparent during the immersion of the test pieces therein. However, those immersed in the conventional bath were interspersed with nickel on the surface and this bath produced dark-colored precipitates during the coating operation.

## EXAMPLE 4

The procedure of Example 1 was repeated, but using polystyrol test pieces instead of the ABS resin ones and using the following etching solution and conventional and novel baths under the following operational conditions:

Etching solution:

|                                             |        |     |
|---------------------------------------------|--------|-----|
| Concentrated H <sub>2</sub> SO <sub>4</sub> | cc./l. | 860 |
| Phosphoric acid (85%)                       | cc./l. | 50  |
| Water                                       | cc./l. | 90  |
| Potassium dichromate                        | g./l.  | 17  |
| Palladium sulphate                          | g./l.  | 9   |
| Temp. of the solution                       | °C.    | 25  |
| Time of immersion                           | min.   | 5   |

## CHEMICAL NICKEL PLATING BATHS

|                                     | Conventional | Novel |
|-------------------------------------|--------------|-------|
| Nickel chloride, g./l.              | 20           | 20    |
| Sodium hypophosphite, g./l.         | 27           | 27    |
| Sodium succinate, g./l.             | 16           | 16    |
| L-ascorbic acid, g./l.              | None         | 10    |
| Lead acetate, mg./l.                | None         | 5.5   |
| pH of the bath (adjusted with NaOH) | 4.8          | 4.8   |
| Temp. of the bath, °C.              | 65           | 65    |
| Time of immersion, min.             | 5            | 5     |

The results obtained were as follows:

The novel bath deposited nickel on the etched test pieces to form a uniform nickel coating on the entire surface thereof, during which the bath was maintained transparent. In contrast with this, the conventional bath deposited nickel on the etched test pieces so that the surface thereof was dotted with the nickel thus deposited, during which the bath was kept transparent.

## EXAMPLE 5

The procedure of Example 1 was repeated, but using test pieces of polyester (sold under the trademark "Lumi-

75

lar" by Toray Inc., Japan), the following etching solution and novel and conventional baths under the following operational conditions:

Etching operation:

|                        |        |     |
|------------------------|--------|-----|
| Conc. $H_2SO_4$        | cc./l. | 800 |
| Water                  | cc./l. | 200 |
| Chromic acid anhydride | g./l.  | 10  |
| Palladium sulfate      | g./l.  | 0.5 |
| Temp. of the solution  | ° C.   | 60  |
| Time of immersion      | min.   | 20  |

CHEMICAL NICKEL PLATING BATHS

|                             | Conventional bath | Novel bath |
|-----------------------------|-------------------|------------|
| Nickel chloride, g./l.      | 60                | 60         |
| Sodium hypophosphite, g./l. | 20                | 20         |
| Citric acid, g./l.          | 100               | 100        |
| Ammonium chloride, g./l.    | 50                | 50         |
| Ascorbic acid, g./l.        | None              | 10         |
| Lead nitrate, mg./l.        | None              | 7          |
| pH (adjusted by NaOH)       | 9                 | 9          |
| Temp. of the bath, ° C.     | 56                | 50         |
| Time of immersion, min.     | 5                 | 5          |

The test pieces from the novel bath had a uniform nickel coating formed all over the etched surface thereof and the bath was kept limpid during the test. On the other hand, those from the conventional bath had no nickel coating and the bath formed a dark-colored precipitate.

EXAMPLE 6

The procedure of Example 1 was repeated, but using test pieces of polypropylene (sold under the trademark "Noblen MM2A" by Mitsubishi Yuka Inc., Japan), the following etching solution and novel and conventional baths under the following operational conditions:

Etching solution:

|                           |        |     |
|---------------------------|--------|-----|
| Conc. $H_2SO_4$           | cc./l. | 500 |
| Water                     | cc./l. | 500 |
| Chromic acid anhydride    | g./l.  | 15  |
| Sodium palladium chloride | g./l.  | 1   |
| Temp. of the solution     | ° C.   | 80  |
| Time of immersion         | min.   | 30  |

CHEMICAL NICKEL PLATING BATHS

|                             | Conventional bath | Novel bath |
|-----------------------------|-------------------|------------|
| Nickel sulphate, g./l.      | 50                | 50         |
| Sodium hypophosphite, g./l. | 20                | 20         |
| Sodium acetate, g./l.       | 10                | 10         |
| Ascorbic acid, g./l.        | None              | 30         |
| Lead acetate, mg./l.        | None              | 5          |
| pH (adjusted by NaOH)       | 5                 | 5          |
| Temp. of the bath, ° C.     | 50                | 50         |
| Time of immersion, min.     | 5                 | 5          |

8  
EXAMPLE 7

The procedure of Example 1 was repeated, but using the following etching solution and conventional and novel baths under the following operational conditions:

Etching solution:

|                        |        |     |
|------------------------|--------|-----|
| Concentrated $H_2SO_4$ | cc./l. | 500 |
| Water                  | cc./l. | 500 |
| Chromic acid anhydride | g./l.  | 15  |
| Palladium chloride     | g./l.  | 0.5 |
| Temp. of the solution  | ° C.   | 60  |
| Time of immersion      | min.   | 15  |

CHEMICAL NICKEL PLATING BATHS

|                             | Conventional (Bath A <sub>1</sub> ) | Novel (Bath D <sub>1</sub> ) |
|-----------------------------|-------------------------------------|------------------------------|
| Nickel chloride, g./l.      | 20                                  | 20                           |
| Sodium hypophosphite, g./l. | 15                                  | 15                           |
| Adipic acid, g./l.          | 15                                  | 15                           |
| Sodium L-ascorbate, g./l.   | 10                                  | 10                           |
| Lead acetate, mg./l.        | 3.7                                 | 3.7                          |
| pH (Adjusted by NaOH)       | 6                                   | 6                            |
| Temp. of the bath, ° C.     | 60                                  | 60                           |
| Time of immersion, min.     | 5                                   | 5                            |

The results obtained were that the novel bath deposited nickel on the test pieces thereby forming a uniform nickel coating over the entire surface thereof while keeping the bath transparent, whereas the conventional bath deposited no nickel while forming a dark-colored precipitate.

Experiment 1

For comparison a test was made by repeating the procedure of Example 7, but using a conventional bath A<sub>1</sub>, a novel bath D<sub>1</sub>, a bath B<sub>1</sub> prepared by adding 10 g./l. of sodium L-ascorbate to a bath A<sub>1</sub>, a bath C<sub>1</sub> prepared by adding 3.7 mg./l. of lead acetate to a bath A<sub>1</sub>, respectively. In the coating step, after the etching step, of the test, test pieces to be coated were treated in such a manner that one test piece was immersed in 200 cc. of the bath for a predetermined period of time (5 min. in this case) before another was in turn immersed under the same conditions as above, in order to investigate the state of a nickel coating formed on the test pieces and the change in appearance of the bath. A set of the twenty test pieces P<sub>1</sub>-P<sub>20</sub> (65 mm. x 40 mm. x 3 mm.) of ABS resin were prepared for use in each of the baths.

The experiment showed that a satisfactory result was obtained only with the novel bath D<sub>1</sub>. The detailed results are shown in the following Table 1.

TABLE 1

Baths used

| State of coating formed and change in appearance of bath | Bath A <sub>1</sub>              |                              | Bath B <sub>1</sub>              |                              | Baths C <sub>1</sub>             |                              | Bath D <sub>1</sub>              |                              |
|----------------------------------------------------------|----------------------------------|------------------------------|----------------------------------|------------------------------|----------------------------------|------------------------------|----------------------------------|------------------------------|
|                                                          | State of coating formed, percent | Change in appearance of bath | State of coating formed, percent | Change in appearance of bath | State of coating formed, percent | Change in appearance of bath | State of coating formed, percent | Change in appearance of bath |
| Test pieces used:                                        |                                  |                              |                                  |                              |                                  |                              |                                  |                              |
| P <sub>1</sub>                                           | 0                                | None                         | 0                                | Decomposed                   | 0                                | None                         | 100                              | None                         |
| P <sub>2</sub>                                           | 0                                | do                           | 0                                | do                           | 0                                | do                           | 100                              | Do.                          |
| P <sub>3</sub>                                           | 0                                | do                           | 20                               | do                           | 100                              | do                           | 100                              | Do.                          |
| P <sub>4</sub>                                           | 0                                | Decomposed                   | 80                               | do                           | 100                              | do                           | 100                              | Do.                          |
| P <sub>5</sub>                                           |                                  |                              | 50                               | do                           | 100                              | do                           | 100                              | Do.                          |
| P <sub>6</sub> -P <sub>15</sub>                          |                                  |                              | 20                               | Decomposed                   | 100                              | do                           | 100                              | Do.                          |
| P <sub>16</sub> -P <sub>20</sub>                         |                                  |                              |                                  |                              |                                  |                              |                                  |                              |

NOTE.—0%: Test pieces were coated with no or very little nickel; 20%, 50% and 80%: Test pieces were coated with nickel on approximately 20%, 50% and 80% of the surface, respectively. 100%: Test pieces were coated with nickel uniformly on the entire surface.

The test pieces from the novel bath had a nickel coating formed all over the surface thereof and the bath remained limpid during the test, while those from the conventional bath had a nickel coating formed on about half the surface thereof and the bath formed a dark-colored precipitate.

Table 1 indicates the following:

(1) In case of the bath A<sub>1</sub>:

P<sub>1</sub> to P<sub>4</sub> (pieces Nos. 1 to 4) were coated with no or very little nickel. The bath decomposed while P<sub>4</sub> was immersed therein, thereby making it impossible to continue the test any further.

(2) In case of the bath B<sub>1</sub>:

P<sub>1</sub> was hardly coated with nickel while the bath decomposed, thereby making it impossible to continue the test any further.

(3) In case of the bath C<sub>1</sub>:

P<sub>1</sub> and P<sub>2</sub> were hardly coated with nickel, P<sub>3</sub> to P<sub>5</sub> were coated with nickel on 20%, 80% and 50% of the surface, respectively, and P<sub>6</sub>–P<sub>15</sub> were coated with nickel on 20%, on the average, of the surface, respectively. The

## Experiment 2

For comparison, the same procedure as in Example 8 was repeated, but using a bath A<sub>2</sub>, a bath B<sub>2</sub> prepared by adding 7 g./l. of sodium L-ascorbate to a bath A<sub>2</sub>, a bath C<sub>2</sub> prepared by adding 7 mg./l. of lead nitrate to a bath A<sub>2</sub>, and a bath D<sub>2</sub>, respectively. In this comparison test, 200 cc. of each of the baths were used and a set of the twenty test pieces (P'<sub>1</sub> to P'<sub>20</sub>) were prepared for use in each of the baths.

The results obtained are shown in Table 2.

TABLE 2

| State of coating formed and change in appearance of bath | Baths used     |                         |                |                         |                |                         |                |  |
|----------------------------------------------------------|----------------|-------------------------|----------------|-------------------------|----------------|-------------------------|----------------|--|
|                                                          | A <sub>2</sub> |                         | B <sub>2</sub> |                         | C <sub>2</sub> |                         | D <sub>2</sub> |  |
| Coating formed, percent                                  | Change of bath | Coating formed, percent | Change of bath | Coating formed, percent | Change of bath | Coating formed, percent | Change of bath |  |
| Test pieces used:                                        |                |                         |                |                         |                |                         |                |  |
| P' <sub>1</sub>                                          | 0 None         | 0 Decomposed            | 0 None         | 100                     | None           | 100                     | None           |  |
| P' <sub>2</sub>                                          | 0 do           | 0 do                    | 0 do           | 100                     | Do             | 100                     | Do             |  |
| P' <sub>3</sub>                                          | 0 do           | 0 do                    | 0 do           | 100                     | Do             | 100                     | Do             |  |
| P' <sub>4</sub>                                          | 0 do           | 0 do                    | 0 do           | 100                     | Do             | 100                     | Do             |  |
| P' <sub>5</sub> –P' <sub>20</sub>                        | (1) Not tested | (1) Not tested          | (1) Not tested | 100                     | Do             | 100                     | Do             |  |

<sup>1</sup> Not tested.

bath decomposed while P<sub>15</sub> was immersed, thereby making the test impossible to be continued any further.

(4) In case of the bath D<sub>1</sub>:

P<sub>1</sub> to P<sub>20</sub> were all coated with nickel uniformly on the entire surface, and the bath did not show any change in appearance throughout the test.

## EXAMPLE 8

The procedure of Example 1 was followed, but using the following etching solution and conventional and novel baths under the following operational conditions:

## Etching solution:

|                                             |        |     |
|---------------------------------------------|--------|-----|
| Concentrated H <sub>2</sub> SO <sub>4</sub> | cc./l. | 800 |
| Water                                       | cc./l. | 200 |
| Chromic acid anhydride                      | g./l.  | 10  |
| Palladium sulfate                           | g./l.  | 0.5 |
| Temp. of the solution                       | °C     | 50  |
| Time of immersion                           | min.   | 10  |

As seen from Table 2, the Baths A<sub>2</sub> and C<sub>2</sub> hardly deposited any nickel on the etched test pieces P'<sub>1</sub> to P'<sub>4</sub> without their changes in appearance, respectively. Thus these baths were not further used in the test. The Bath B<sub>2</sub> completely decomposed without depositing nickel on P'<sub>1</sub> and with a dark-colored precipitate formed when P'<sub>1</sub> was immersed in the bath, while the novel bath D<sub>2</sub> was extremely stable and deposited nickel uniformly on the entire surface of P'<sub>1</sub> to P'<sub>20</sub> without its change in appearance.

## EXAMPLE 9

The procedure of Example 1 was followed, but using the following etching solution and conventional and novel baths under the following operational conditions:

## Etching solution:

|                                                                |        |     |
|----------------------------------------------------------------|--------|-----|
| Conc. H <sub>2</sub> SO <sub>4</sub>                           | cc./l. | 500 |
| Water                                                          | cc./l. | 500 |
| Potassium dichromate                                           | g./l.  | 10  |
| Sodium palladium chloride (Na <sub>2</sub> PdCl <sub>4</sub> ) | g./l.  | 1   |
| Temp. of the solution                                          | °C     | 60  |
| Time of immersion                                              | min.   | 10  |

## CHEMICAL NICKEL PLATING BATHS

| CHEMICAL NICKEL PLATING BATHS          |                                 |    |
|----------------------------------------|---------------------------------|----|
| Conventional<br>(Bath A <sub>3</sub> ) | Novel<br>(Bath D <sub>3</sub> ) |    |
| Nickel sulfate, g./l.                  | 16                              | 16 |
| Sodium hypophosphite, g./l.            | 11                              | 11 |
| Citric acid, g./l.                     | 10                              | 10 |
| Borax, g./l.                           | 6                               | 6  |
| Sodium L-ascorbate, g./l.              | 0                               | 7  |
| Lead nitrate, mg./l.                   | 9                               | 9  |
| pH (adjusted by NaOH)                  | 40                              | 40 |
| Temp. of the bath, °C                  | 40                              | 40 |
| Time of immersion, min.                | 3                               | 3  |

|                                                  | Conventional<br>(Bath A <sub>3</sub> ) | Novel<br>(Bath D <sub>3</sub> ) |
|--------------------------------------------------|----------------------------------------|---------------------------------|
| Nickel sulfate, g./l.                            | 20                                     | 20                              |
| Sodium hypophosphite, g./l.                      | 15                                     | 15                              |
| Sodium succinate, g./l.                          | 15                                     | 15                              |
| Sodium L-ascorbate, g./l.                        | 0                                      | 30                              |
| Lead acetate, mg./l.                             | 0                                      | 5                               |
| pH (adjusted by H <sub>2</sub> SO <sub>4</sub> ) | 4                                      | 4                               |
| Temp. of the bath, °C                            | 60                                     | 60                              |
| Time of immersion, min.                          | 3                                      | 3                               |

The results obtained were that the conventional bath hardly deposited any nickel on the etched test pieces with a dark-colored precipitate formed therein, whereas the novel one deposited nickel uniformly on the surface of the etched test pieces while keeping the bath transparent.

## Experiment 3

The results obtained showed that the conventional bath deposited no nickel on the etched pieces without change in appearance of the bath (transparent), while the novel bath deposited nickel on the etched test pieces uniformly on the entire surfaces without change in appearance of the bath (transparent).

A comparative test was made in the same manner as in Example 9, but using each of a conventional bath A<sub>3</sub>, a bath B<sub>3</sub> prepared by adding 30 g./l. of sodium L-ascorbate to a bath A<sub>3</sub>, and a novel bath D<sub>3</sub>. In this experiment 200 cc. of each of the baths were used and a set of the test pieces (P''<sub>1</sub>–P''<sub>20</sub>) were prepared for use

in each of the baths, as in the other experiments. The results obtained are indicated in Table 3.

TABLE 3

| State of coating formed and change in appearance of bath | Bath used               |                |                         |                |
|----------------------------------------------------------|-------------------------|----------------|-------------------------|----------------|
|                                                          | A <sub>3</sub>          |                | B <sub>3</sub>          |                |
|                                                          | Coating formed, percent | Change of bath | Coating formed, percent | Change of bath |
| Test pieces used:                                        | 20                      | None           | 100                     | None           |
| P'' <sub>1</sub>                                         |                         | Decomposed     |                         | 0              |
| P'' <sub>2</sub>                                         |                         |                | 0                       | do             |
| P'' <sub>3</sub>                                         |                         |                | 0                       | do             |
| P'' <sub>4</sub>                                         |                         |                | 0                       | do             |
| P'' <sub>5</sub> -P'' <sub>20</sub>                      |                         |                | 0                       | do             |

The results shown in Table 3 tend to be almost similar to those obtained from Experiments 1 and 2.

Table 3 indicates the following:

The bath A<sub>3</sub> deposited nickel on approximately 20% of the surface of P''<sub>1</sub> and it decomposed while P''<sub>2</sub> was immersed therein.

The bath B<sub>3</sub> deposited nickel uniformly on the entire surface of P''<sub>1</sub> while it was made turbid, and it decomposed when P''<sub>2</sub> was immersed.

The bath C<sub>3</sub> deposited nickel in fine spot form on each of P''<sub>1</sub> to P''<sub>20</sub> without change of the bath in appearance.

15

## EXPERIMENT 4

For comparison, the procedure of Example 10 was repeated, but using a bath A<sub>4</sub>, a bath B<sub>4</sub> prepared by adding 10 g./l. of sodium L-ascorbate to a bath A<sub>4</sub>, a bath C<sub>4</sub> prepared by adding 5.5 mg./l. of lead acetate to a bath A<sub>4</sub>, and a bath D<sub>4</sub>, respectively. In this experiment, 200 cc. of each of the baths were used and twenty test pieces prepared for each of the baths, as in the previously-mentioned experiments.

The results obtained are indicated in the following table.

TABLE 4

| State of coating formed and change in appearance of bath | Bath used               |                |                         |                |
|----------------------------------------------------------|-------------------------|----------------|-------------------------|----------------|
|                                                          | A <sub>4</sub>          |                | B <sub>4</sub>          |                |
|                                                          | Coating formed, percent | Change of bath | Coating formed, percent | Change of bath |
| Test pieces used:                                        |                         |                |                         |                |
| P'' <sub>1</sub>                                         | 100                     | None           | 100                     | None           |
| P'' <sub>2</sub>                                         | 100                     | do             | 100                     | do             |
| P'' <sub>3</sub>                                         | 100                     | do             | 50                      | do             |
| P'' <sub>4</sub>                                         |                         | Decomposed     | 50                      | do             |
| P'' <sub>5</sub> -P'' <sub>20</sub>                      |                         |                | 50                      | do             |

The bath D<sub>3</sub> deposited nickel uniformly on the entire surface of each of P''<sub>1</sub> to P''<sub>20</sub> while it was quite limpid.

## EXAMPLE 10

Test pieces used: Styrol resin plaques 45 mm. x 40 mm. x 1.5 mm.

45

Etching solution:

|                                      |        |     |
|--------------------------------------|--------|-----|
| Conc. H <sub>2</sub> SO <sub>4</sub> | cc./l. | 860 |
| Phosphoric acid                      | cc./l. | 50  |
| Water                                | cc./l. | 90  |
| Potassium dichromate                 | g./l.  | 17  |
| Palladium sulfate                    | g./l.  | 9   |
| Temp. of the solution                | ° C.   | 25  |
| Time of immersion                    | min.   | 5   |

50

50

55

55

55

60

60

65

65

## CHEMICAL NICKEL PLATING BATHS

|                                                  | Conventional (Bath A <sub>4</sub> ) | Novel (Bath D <sub>4</sub> ) |
|--------------------------------------------------|-------------------------------------|------------------------------|
| Nickel chloride, g./l.                           | 20                                  | 20                           |
| Sodium hypophosphite, g./l.                      | 27                                  | 27                           |
| Sodium succinate, g./l.                          | 16                                  | 16                           |
| Sodium L-ascorbate, g./l.                        | 0                                   | 10                           |
| Lead acetate, mg./l.                             | 0                                   | 5.5                          |
| pH (adjusted by H <sub>2</sub> SO <sub>4</sub> ) | 4.8                                 | 4.8                          |
| Temp. of the bath, ° C.                          | 65                                  | 65                           |
| Time of immersion, min.                          | 5                                   | 5                            |

The results obtained are as follows:

The conventional bath deposited nickel on the entire surface of only some test pieces used at the early stage of the plating operation, while the bath formed a dark-colored precipitate shortly after the start of the plating operation. On the other hand, the novel bath deposited

70

75

75

nickel uniformly on the entire surface of each of the test pieces used while it remained limpid.

## 12

## 13

of a nickel salt, 3-40 g./l., calculated as hypophosphite ion, of a hypophosphite and 5-100 g./l. of another organic acid.

2. A process according to claim 1 wherein the palladium salt is selected from the group consisting of palladium chloride, palladium sulfate and sodium palladium chloride.

3. A process according to claim 1 wherein the nickel salt is selected from the group consisting of nickel sulphate and nickel chloride, the hypophosphite is sodium hypophosphite and said organic acid is selected from the group consisting of short-chain mono-, di- and tricarboxylic acids, hydroxycarboxylic acids, and aminocarboxylic acids.

4. A process according to claim 1 wherein said palladium salt is present in said aqueous etching solution in an amount of from 0.2-5 g./l., calculated as palladium.

5. A process according to claim 1 wherein said plating bath contains 10 to 30 g./l., calculated as ascorbic acid,

## 14

of said ascorbic acid and its salts and 2-7 mg./l. of said lead compound, calculated as lead ion.

6. A process according to claim 1 wherein said second reducing agent is ascorbic acid or the sodium salt thereof.

5 7. Plated product manufactured by the process of claim 1.

## References Cited

## UNITED STATES PATENTS

|    |           |        |                  |          |
|----|-----------|--------|------------------|----------|
| 10 | 3,597,267 | 8/1971 | Mallory et al.   |          |
|    | 3,437,507 | 4/1969 | Jensen           | 106-1 X  |
|    | 3,459,563 | 8/1969 | Terashima et al. | 106-1    |
|    | 3,488,166 | 1/1970 | Kovac et al.     | 117-47 X |
|    | 3,553,085 | 1/1971 | Heymann          | 117-47 X |

15 ALFRED L. LEAVITT, Primary Examiner

J. A. BELL, Assistant Examiner

U.S. CL. X.R.

20 106-1; 117-160 R; 204-30